# EUROPEAN PATENT SPECIFICATION

(11) **EP 0 391 653 B1**
(45) Date of publication and mention of the grant of the patent: **02.03.1994**
(21) Application number: 90303538.4
(22) Date of filing: 02.04.1990
(51) Int. Cl.: C10M 141/08, C10M 141/10, C10M 141/12, C10M 167/00

(54) **Lubricant compositions**
Schmiermittelzusammensetzungen
Compositions lubrifiantes

(30) Priority: 03.04.1989 GB 8907474
(43) Date of publication of application: 10.10.1990
(73) Proprietor: ETHYL PETROLEUM ADDITIVES LIMITED, Bracknell, Berkshire RG12 2UW (GB)
(72) Inventor: Thomas, Arthur Samuel, Swansea, SA3 3DN, Wales (GB); Macpherson, Ian, Windsor, Berkshire SL4 4PE (GB); Richardson, Clive Ralph, Wokingham, Berkshire RG11 1TE (GB)
(74) Representative: Collier, Jeremy Austin Grey

(56) References cited:
- EP-A- 0 086 513
- EP-A- 0 094 144
- WO-A-86/05508
- US-A- 3 013 970
- US-A- 3 389 083
- US-A- 3 398 095
- US-A- 4 263 155
- DATABASE WPI, no. 68-34654q, Derwent Publications Ltd, London, GB;& DD-A-63 835 (EGER REMETH)
- DATABASE WPI, no. 80-80939c, Derwent Publications Ltd, London, GB;& DD-A-144 072 (F. LOHRMANN)

## Description

This invention relates to lubricating fluid compositions, and in particular to gear oils and to additives therefor.

High performance gear oils usually consist of a major amount of mineral oil or synthetic base stock and a minor amount of suitable additives including in particular a sulphur-containing extreme pressure or anti-wear agent. Such sulphur-containing materials are highly effective in promoting the extreme pressure and anti-wear properties of the oil and may also have valuable anti-oxidant properties. However, such sulphur-containing materials are detrimental to the environment, may cause undesirable odour, and can lead to corrosion of the metal parts with which they come in contact, especially parts containing copper.

Gear oils, for example the oils used in the gear boxes and differentials of motor vehicles, and other mechanisms involving metal on metal, for example steel on steel or steel on bronze, acting parts, are required to protect the metal surfaces and particularly the teeth of the gears. Typically, such oils remain in use for long periods without being changed. In addition to providing general lubrication, the fluid protects the loaded metal parts such as the gear teeth from damage. Gear oils are customarily tested for their ability to protect gear teeth from damage such as wear and pitting for long periods. In one system for testing such oils a gear train is run under conditions of variable and very heavy stress until the gears fail. The length of time before such failure takes place, or the wear of the gear teeth (as measured by the iron content of the fluid) becomes excessive, provides a measure of the effectiveness of the gear oil. Some current gear oils provide a measure of protection in this respect, but still further improvement is desirable.

There is therefore a need for gear lubricating oils which provide better protection of the gears and/or which contain reduced sulphur content, and for additive systems for such oils.

We have now discovered that the performance of sulphur-containing gear oils may be improved, and/or the sulphur content of such oils reduced, by incorporating in the oils a combination of a weak acid and an amine. Both acids and amines have heretofore been used in lubricating oil compositions, but the known compositions do not achieve the advantages of the present invention. For example, United States Patent No. 3398095 discloses oils containing sulphurized carboxylic acid in combination with acids and amines as so-called "vapour space inhibitors". Such oils are stated to achieve excellent corrosion inhibition for ferrous metals. They are not however suitable as gear oils. United States Patent No. 4615818 discloses that lubricant compositions comprising an oil-soluble sulphurized organic compound may be improved, so as to reduce emission of volatile sulphur compounds, by inclusion of a hindered organic amine and preferably a carboxylic acid. There is, however, no suggestion that the performance of gear oils can be improved by inclusion of the hindered amine with or without the carboxylic acid. In fact the compositions disclosed in this patent do not improve the performance of gear oils.

US 4,792,410 discloses an oil based manual transmission lubricant containing a borated overbased alkali metal or alkaline earth metal salt and a friction modifier which may be inter alia a fatty amine or a sulfurised olefin.

The present invention accordingly provides a lubricant composition comprising a lubricant, 1.7 to 20% by weight of one or more sulphur-containing extreme pressure or anti-wear agents including at least one such agent containing sulphur bound directly to carbon or to more sulphur, from 0.1 to 10% by weight of a weak acid having a pKa of greater than 2 and from 0.05 to 10% by weight of an amine, the said percentages being based on the weight of the lubricant, the amount of the said acid being from 0.2 to 2 equivalents per equivalent of the said amine, and the salt of the said acid with said amine being soluble in the said lubricant in which the molar ratio of the sulphur in the said sulphur-containing extreme pressure or antiwear agents to the amino nitrogen in the said amine is from 40:1 to 5:1. The proportion of the said acid is usually from 0.67 to 1.25 equivalents per equivalent of the said amine.

The lubricant may be a mineral oil, a synthetic oil, a natural oil such as a vegetable oil, or a mixture thereof, e.g. a mixture of a mineral oil and a synthetic oil. Suitable mineral oils include those of appropriate viscosity refined from crude oil of any source including Gulf Coast, Midcontinent, Pennsylvania, California, Alaska, Middle East, North Sea and the like. Standard refinery operations may be used in processing the mineral oil.

Synthetic oils include both hydrocarbon synthetic oils and synthetic esters. Useful synthetic hydrocarbon oils include liquid alpha olefin polymers of appropriate viscosity. Especially useful are hydrogenated liquid oligomers of C₆-C₁₆ alpha-olefins, such as hydrogentated or unhydrogenated alpha-decene trimer. Alkyl-benzenes of appropriate viscosity, e.g. didodecylbenzene, can also be used.

Useful synthetic esters include the esters of monocarboxylic and polycarboxylic acids with monohydroxy alcohols and polyols. Typical examples are didodecyl adipate, trimethylolpropane tripelargonate, pentaerythritol tetracaproate, di(2-ethylhexyl) adipate, and dilauryl sebacate. Complex esters made from mixtures of mono- and di-carboxylic acids and mono- and/or polyhydric alkanols can also be used.

The compositions of the present invention can be blended into any such lubricant base stocks. The base oil is generally a mineral oil base stock such as, for example, a conventional or solvent-refined paraffinic neutral or bright stock, a hydrotreated paraffinic neutral or bright stock, a naphthenic oil, or a cylinder oil, etc., including both straight run and blended oils. As noted above, synthetic base stocks such as for example poly-alpha-olefins with synthetic diesters in weight proportions (PAO:ester) ranging from about 95:5 to about 50:50, typically about 72:25 can be used. Generally speaking, the base stocks used in automotive gear oils range in viscosity grades from SAE 50 to 250 and preferably from 70 to 140. Suitable automotive gear oils also include cross-grades such as 75W-140, 80W-90, 85W-140, 85W-90, and the like. In general, the base stocks used in industrial gear oils have a viscosity in the range of from about ISO grade 32 to ISO grade 680 and preferably from ISO grade 68 to ISO grade 460.

The new lubricant compositions may be supplied either as finished lubricants ready for use or in the form of an additive package, i.e. a concentrate, which requires dilution with base lubricating fluid before use. As described in more detail below, the lubricant compositions of the invention may contain, in addition to the substances already mentioned, any usual additive for inclusion in such lubricants which is compatible with the sulphur-containing agent and the acid and amine. Examples of such additives are given below.

At least one of the sulphur containing oil soluble extreme pressure or antiwear agents used in the compositions of the present invention contains sulphur bound directly to carbon or to more sulphur and in the preferred compositions of the invention the sulphur atoms in the sulphur containing species are highly active.

A very wide variety of sulphur-containing oil-soluble extreme pressure or anti-wear agents may be used in the compositions of the invention, and any known such agents may in principle be used. Usually the agent used contains highly active sulphur, i.e. sulphur in an amount and structural configuration such that it is capable of causing visually observable corrosive pitting of one or more gear tooth surfaces in the standard planetary spur gear test when conducted in the way described below for up to 40 hours. Examples of such agents are sulphurised olefins, sulphurised esters, sulphurised fatty acids, dialkylpolysulphides, diarylpolysulphides, dialkarylpolysulphides, sulphur, and sulphurised oils such as sulphurised sperm oil or sulphurised lard oil.

Whilst pitting in the standard planetary spur gear test is probably the best criterion for determining for the purpose of the present invention whether a sulphur-containing extreme pressure or anti-wear agent is or is not "highly active", another procedure which correlates reasonably well with the spur gear test can be used for this purpose. The alternative procedure is a copper coupon corrosion test which is conducted as follows: A copper coupon approximately 70 X 15 mm and about 1.25 mm in thickness is cleaned with steel wool (0000 grade), washed with heptane, and then with acetone, dried, and weighed to the nearest 0.1 mg. The cleaned coupon is placed in a test tube and covered completely with the composition to be tested, and the system is heated to 125°C in an oil bath maintained at this temperature. After holding the system at 125°C for three hours, the copper coupon is removed from the test tube, rinsed with heptane and then with acetone. The dried coupon is then rubbed with a paper towel moistened with acetone to remove any surface flakes formed by copper corrosion. The coupon is then air-dried and weighed to the nearest 0.1 mg. The difference in weight between the initial copper coupon and the coupon after the test represents the extent to which the copper has been corroded under the test conditions: the larger the weight difference, the greater the copper corrosion, and thus the more active the sulphur compound. For the purposes of this invention a sulphur-containing extreme pressure or anti-wear agent is regarded as "highly-active" if the coupon weight loss in the above test is above 50 milligrams. If the weight loss is from 30 to 50 milligrams, the agent should be subjected to the planetary spur gear test in order to determine whether it is "highly active" or not.

Generally speaking, sulphur-containing compounds which possess a linkage of two sulphur atoms (i.e., -S-S-) or four or more sulphur atoms (e.g., -S-S-S-S-, -S-S-S-S-S-, etc.) tend to be "highly active" in the sense used herein. In some cases a product from one manufacturer, for example sulphurised isobutene, may be "highly active" whereas a similar product from another manufacturer may not be "highly active". Thus in cases where the activity of a given sulphur-containing extreme pressure or anti-wear agent is not known with certainty, it is desirable to perform a test such as the planetary spur test to ascertain whether it is "a highly active" material in the sense of the present invention.

One preferred class of such agents is made by reacting an olefin such as isobutene with sulphur. The product, e.g. sulphurised isobutene, typically has a sulphur content of about 10 to about 50%, preferably 30 to 50%, by weight. A wide variety of other olefins or saturated hydrocarbons may be used in place of the isobutene.

Another example of a sulphur-containing extreme pressure agent which may be used in the compositions of the invention is sulphur.

The compositions of the present invention may contain, as an extreme pressure or anti-wear agent, an ester of a pentavalent acid of phosphorus, such as a fully or partially esterified phosphoric, phosphonic or pyrophosphoric acids or a sulphur-containing analog thereof. Such compounds have the formula:
wherein each of R¹, R² and R³ is, independently, hydrogen or a hydrocarbyl group, provided that at least one of R¹, R² and R³ is hydrocarbyl, and each X is oxygen or sulphur, at least one X being sulphur. Most preferred are compounds of the formula
where at least 95 percent of the R¹ groups are hydrocarbyl groups, the balance, if any, being hydrogen atoms, and R² and R³, when hydrocarbyl, can be aromatic, cycloaliphatic, and/or aliphatic hydrocarbon groups, or any combination of these. Preferably R¹, R² and R³ are saturated or substantially saturated aliphatic, cycloaliphatic or polycycloaliphatic groups, such as alkyl, alkenyl, cycloalkyl, cycloalkenyl, cycloalkylalkyl, cycloalkylalkenyl, cycloalkenylalkyl, cycloalkenylalkenyl, and the like. As far as chain length or carbon atom content is concerned, the only requirement is that the hydrocarbyl groups are such that the compound is soluble in the base oil to at least the desired use concentration at ambient temperatures. The hydrocarbyl groups can contain functional substituents or non-hydrocarbon component groups which do not materially alter the predominantly hydrocarbon character of the hydrocarbyl groups themselves.

Examples of sulphur-containing extreme pressure agents where the sulphur is not bound directly to carbon or sulphur include the sulphur- and phosphorus-containing additives especially the thiophosphates and dithiophosphates, e.g. zinc dialkyl or diaryl dithiophosphates or trihydrocarbyldithiophosphates, customarily included in lubricant compositions as extreme pressure or anti-wear agents.

Because of the toxicity and disagreeable odour of hydrogen sulphide, it is desirable to use a highly active sulphur-containing extreme pressure or anti-wear agent that yields less than 500 ppm of vapour space H₂S when heated by itself for one week at 65°C.

The proportion of sulphur-containing extreme pressure or antiwear agents included in the compositions of the invention is preferably such that the molar ratio of the sulphur in the said sulphur-containing extreme pressure or anti-wear agents to the amino nitrogen in the amine or amino acid is from 40:1 to 5:1, and is typically 1.7 to 10% by weight, usually 2-4%, based on the weight of the lubricant.

In calculating the proportion of sulphur, the total sulphur content of the extreme pressure or antiwear agents should be taken into account, even though some of the sulphur in the agents may not qualify as "highly active" in the strict sense explained above.

The new compositions preferably contain a phosphorus-containing extreme pressure or anitwear agent. As already indicated the sulphur-containing agents may contain phosphorus, or a separate phosphorus-containing agent may be used with the sulphur-containing agents (which may themselves, contain phosphorus). Such separate phosphorus-containing agents include derivatives of phosphorus oxyacids and of polyphosphorus oxyacids such as phosphites, phosphates and pyrophosphates, and especially their oil-soluble esters, acid esters and amine salts. Preferably a mono- or di-hydrocarbyl phosphite or phosphate or a mixture thereof is used, where the hydrocarbyl groups may be alkyl, alkenyl, phenyl, alkylphenyl or dialkylphenyl. Examples of suitable esters are monomethyl, dimethyl, mono-n-butyl, di-n-butyl, mono-isobutyl, di-isobutyl, monoamyl, diamyl, di-n-octyl, di-(2-ethyl-n-hexyl), monooleyl, dioleyl, monophenyl, diphenyl and di(dodecylphenyl) phosphite and phosphate, and their amine salts. Such phosphorus-containing agents are usually included in the new compositions in a proportion of 0.01 to 3.5% based on the weight of the lubricant.

The compositions of the invention may also contain an alkali metal borate, e.g. sodium or potassium borate, e.g. in a proportion of 0.5 to 8% by weight of the lubricant.

The acid used in the new compositions is a weak acid, having a pKa of greater than about 2.0, and is usually a carboxylic acid in which one or more carboxyl groups are attached to a hydrocarbon radical of 1 to 100, preferably 2 to 36 carbon atoms. Other weak acids, e.g. a boric acid such as H₃BO₃ or metaboric acid, may also be used, e.g. in a amount from 0.1 to 8.0% by weight of the lubricant. Examples of suitable acids are alkanoic and alkenoic mono-, di- or poly-carboxylic acids of 1 to 100, preferably 2 to 54, carbon atoms, e.g. acetic acid, n-octanoic acid, decanoic acid, myristic acid, oleic acid, linoleic acid, tetrapropenylsuccinic acid, azelaic acid, or dimerised or trimerised linoleic acid. The acid used must be such as to form an oil-soluble salt with the amine used. Acyclic monocarboxylic acids are preferred.

Any amine may potentially be used in the compositions of the present invention. Preferred amines are aliphatic mono and polyamines containing 2 to 22 carbon atoms per molecule. Primary, secondary and tertiary amines are all suitable. Especially preferred amines are linear or branched aliphatic, cycloaliphatic or ethylenically unsaturated aliphatic amines of 6 to 22 carbon atoms, e.g. n-octylamine, oleylamine, or cyclohexylamine, polyethylene polyamines such as triethylene tetramine, and the tertiary alkyl primary amines sold under the trade names Primene 81-R and Primene JM-T. As already noted, the amine must be capable of forming an oil-soluble salt with the acid used.

The combined proportions of the carboxylic acid and of the amine used may be from 0.15 to 20.0% by weight of the lubricant, preferably 0.15 to 2.0%, and especially about 0.3%, but their respective amounts depend as already indicated on their molecular weights and the mole equivalence of the particular acid and amine used. In relation to the sulphur containing extreme pressure or antiwear agent the total amount of acid plus amine is typically 5 to 300%, preferably 20 to 100%, by weight.

In calculating the proportion of amino nitrogen in the compositions of the present invention, only free amine or amine salified with a weak acid should be taken into account. For example any amine salified with a phosphorus acid such as a dialkyl acid phosphate or phosphite is too tightly bound to be available for securing the improved results of the compositions of the present invention, and thus although such amine salts may be present in the compositions of this invention, the amount of amino nitrogen in such amine salts should not be considered as amino nitrogen in calculating the proportion of the latter in the compositions of the invention.

One measure for determining that the correct proportion of amine has been used in the new compositions in relation to the acid is a determination of the pH of the composition. Since the compositions consist essentially of a solution of various organic compounds normally in an oil which is usually a hydrocarbon oil, the compositions have, in a strict sense, no pH. However, it has been found that if a sample of the composition is diluted in a mixture of methanol and toluene and then assayed with a conventional pH probe as used in aqueous systems, a measurement is obtained which provides a useful measure of the relative proportions of basic and acidic materials present in the composition. Measured in this way, the pH of the compositions of the invention should be in the range of 3 to 10 or preferably of 7 to 9.

The compositions of the invention may contain other additives suitable for use in gear oils, for example:

### Antioxidants

Zinc dialkyldithiophosphates, zinc diaryldithiophosphates, hindered phenols, amines and various organic compounds containing nitrogen, sulphur or phosphorus.

### Antifoamants and demulsification agents

Silicone based fluids, ethylene glycol-propylene glycol condensation products, polyalkylacrylates.

### Dispersants

Polyalkenyl succinimides, succinate esters, N-vinyl-pyrrolidone-methacrylate ester copolymers, fatty acid esters and fatty acid amides, and carboxylic acid derivative compositions (e.g. succinimides, succinic acid esters, succinic acid ester-amides, etc.) that have been post-treated by reaction with one or more post-treating reagents such as boron oxide, boron oxide hydrate, boron halides, boron acids, esters of boron acids, carbon disulphide, hydrogen sulphide, sulphur, sulphur chloride, alkenyl cyanides, carboxylic acid acylating agents (e.g. maleic anhydride, maleic acid, fumaric acid, malic acid, azelaic acid, adipic acid, C1 to C30 alkenyl succinic acids, C1 to C30 alkenylsuccinic anhydrides, etc.), aldehydes, ketones, urea, thiourea, guanidine, dicyandiamide, hydrocarbyl phosphates, hydrocarbyl phosphites, hydrocarbyl thiophosphates, hydrocarbyl thiophosphites, phosphorus sulphides, phosphorus oxides, phosphoric acid, phosphorous acid, hydrocarbyl thiocyanates, hydrocarbyl isocyanates, hydrocarbyl isothiocyanates, epoxides, episulphides, formaldehyde or formaldehyde producing compounds plus phenols, and sulphur plus phenols.

### Detergents

Metal salts of organic salicylates, sulphonates, phenates or phosphonates.

### Viscosity index improvers or pour point depressants

Polyalkylmethacrylates or olefin copolymers.

### Friction Modifiers

Alkyl or alkenyl fatty acid amides, alkyl or alkenyl succinimides, or alkyl or alkenyl phosphonates.

The invention includes within its scope a lubricant additive concentrate comprising 5 to 95% of one or more sulphur-containing extreme pressure or anti-wear agents including at least one such agent containing sulphur bound directly to carbon or to sulphur, from 0.5 to 20% of a weak acid and from 1 to 20% of an amine, and a diluent oil, the said percentages being by weight based on the total weight of the concentrate, the amount of the said acid being from 0.2 to 2 equivalents per equivalent of the said amine in which the molar ratio of the sulphur in said sulphur-containing extreme pressure or anti-wear agents to the amino nitrogen in the said amine is from 40:1 to 5:1.

The compositions of the invention can conveniently be made by modification of existing compositions by adding appropriate amounts of acid and amine thereto.

The following Examples illustrate the invention.

### EXAMPLES 1-3

The ingredients listed below were incorporated in an SAE 80W90 mineral oil of North Sea origin. The percentages by weight of each ingredient in the base oil is given.

These blends contain 12.1 moles of sulphur per mole of amino nitrogen in the n-octylamine salt and 0.77 equivalents of octanoic acid per equivalent of n-octylamine.

### EXAMPLE 4

A lubricating fluid of SAE 90 grade viscosity characteristics was blended with sulphurised isobutylene (2.2% w/w), an alkylamine/alkylphosphate/alkylphosphite/alkylthiophosphate mixture (0.5% w/w), and octanoic acid in a proportion such that there were approximately 135.6 moles of sulphur per mole of said acid. The sulphurised isobutylene itself contained 45% sulphur (w/w). The alkylamine is entirely neutralised by the phosphorus acids present.

This fluid was tested using the planetary spur gear test described below in which it gave 40 hours satisfactory running performance before excessive gear damage was observed. This test was repeated twice giving an average result of 44 hours.

A sample of the fluid described above was then treated with an n-octylamine/n-octanoic acid mixture (in equivalent amounts; 0.3% w/w) and then subjected to the same planetary spur gear test. The fluid contained about 38.2 moles of sulphur per mole of amino nitrogen, apart from the nitrogen sulphurised by the phosphorus acids, and 0.9 equivalents of octanoic acid per equivalent of amino nitrogen. This gave a performance of over 75 hours before excessive gear damage was observed.

### The Planetary Spur Gear Test

In this test a system of spur-type gears is driven under variable and very heavy loads. The lubricating fluid is circulated around the system by a pump and is maintained at between 95°C and 130°C. Samples of the lubricating fluid are removed periodically and analysed for iron content. The test is terminated when excessive wear is recorded either by high iron levels in the oil, or by gear tooth breakage. Lubricating fluids produced in accordance with the present invention are capable of enabling at least 60 and in preferred embodiments over 75 hours of running time in the test.

### EXAMPLE 5

A sample of the first lubricating fluid described in Example 4 was treated with an acetic acid/oleylamine mixture (0.11% w/w acetic acid; 0.54% w/w oleylamine), and then subjected to the planetary spur gear test. The fluid contained approximately 23 moles of sulphur per mole of amino nitrogen, other than that salified by the phosphorus acids, and 0.95 equivalents of acetic acid per equivalent of amino nitrogen. Satisfactory performance of over 60 hours was obtained.

### EXAMPLE 6

A sample of the first lubricating fluid described in Example 4 was treated with a mixture of tetrapropenylsuccinic acid and triethylenetetramine (0.22% w/w acid and 0.04% w/w amine), and then subjected to the planetary spur gear test. The fluid contained approximately 29.4 moles of sulphur per mole of amino nitrogen other than that salified by the phosphorus acids. Satisfactory performance over 60 hours was obtained.

## Claims

1. A lubricant composition comprising a lubricant, 1.7 to 20% by weight of one or more sulphur-containing extreme pressure or anti-wear agents including at least one such agent containing sulphur,bound directly to carbon or to more sulphur from 0.1 to 10% by weight of a weak acid having a pKa of greater than 2 and from 0.05 to 10% by weight of an amine, the said percentages being based on the weight of the lubricant, the amount of the said acid being from 0.2 to 2 equivalents per equivalent of the said amine, and the salt of the said acid with said amine being soluble in the said lubricant in which the molar ratio of the sulphur in the said sulphur-containing extreme pressure or antiwear agents to the amino nitrogen in the said amine is from 40:1 to 5:1.

2. A composition according to claim 1 containing 0.67 to 1.25 equivalents of the said acid per equivalent of the said amine.

3. A composition according to claim 1 or 2 containing 1.7 to 10% by weight of the lubricant of the said sulphur-containing extreme pressure or anti-wear agent.

4. A composition according to any of claims 1 to 3 in which the sulphur atoms in the or a sulphur-containing extreme pressure or antiwear agent are highly active.

5. A composition according to any one of claims 1 to 4 in which the or a said sulphur-containing extreme pressure or anti-wear agent contains 30 to 50% by weight of sulphur.

6. A composition according to claim 5 in which the said sulphur-containing extreme pressure or antiwear agent containing sulphur bound directly to carbon or to more sulphur is sulphur, a sulphurized olefin, sulphurized ester, sulphurized fatty acid, or dialkylpolysulphide.

7. A composition according to claim 6 in which the said agent is sulphurized isobutene.

8. A composition according to any of claims 1 to 7 in which at least one of the sulphur-containing extreme pressure or anti-wear agents is a dialkyldithiophosphate or another sulphur-containing phosphite or phosphite ester or salt.

9. A composition according to any of claims 1 to 8 which also contains 0.01 to 3.5% by weight of the lubricant of a phosphorus-containing extreme pressure or anti-wear agent.

10. A composition according to claim 9 in which the said phosphorus-containing agent is a mono- or di-hydrocarbyl phosphate or a mixture thereof wherein the said hydrocarbyl is alkyl, alkenyl, phenyl, alkylphenyl or dialkylphenyl.

11. A composition according to any one of claims 1 to 10 which also contains 0.1 to 8% by weight of the lubricant of an alkali metal borate.

12. A composition according to any one of claims 1 to 11 in which the amine is a linear or branched aliphatic, cycloaliphatic, or linear or branched ethylenically unsaturated aliphatic amine of 6 to 22 carbon atoms, or a polyethylene polyamine.

13. A composition according to claim 12 in which the amine is a tertiary alkyl primary amine, n-octylamine, oleylamine, or triethylenetetramine.

14. A composition according to any one of claims 1 to 13 in which the said acid is a carboxylic acid.

15. A composition according to claim 14 in which the said acid is an alkanoic or alkenoic mono- or di- or polycarboxylic acid of 2 to 54 carbon atoms.

16. A composition according to claim 15 in which the said acid is acetic acid, n-octanoic acid, decanoic acid, myristic acid, oleic acid, linoleic acid, tetrapropenylsuccinic acid, azelaic acid, or dimerized or trimerized linoleic acid.

17. A composition according to any one of the preceding claims which also contains one or more of antioxidants, antifoamants or demulsification agents, dispersants, detergents, viscosity index improvers, pour point depressants and friction modifiers.

18. A lubricant additive concentrate comprising 5 to 95% of one or more sulphur-containing extreme pressure or anti-wear agents including at least one such agent containing sulphur bound directly to carbon or to more sulphur, from 0.5 to 20% of a weak acid having a pKa of greater than 2 and from 1 to 20% of an amine, and a diluent oil, the said percentages being by weight based on the total weight of the concentrate, the amount of the said acid being from 0.2 to 2 equivalents per equivalent of the said amine in which the molar ratio of the sulphur in said sulphur-containing extreme pressure or anti-wear agents to the amino nitrogen in the said amine is from 40:1 to 5:1.

19. A lubricant additive concentrate according to claim 18 which also contains 1 to 50% of one or more phosphorus-containing extreme pressure or anti-wear agents.

## Patentansprüche

1. Schmiermittelzusammensetzung, dadurch gekennzeichnet, daß sie ein Schmiermittel, von 1,7 bis 20 Gew.-% eines oder mehrerer Schwefel enthaltender Höchstdruckadditive oder Verschleißminderer, eingeschlossen mindestens ein solches Mittel, welches Schwefel direkt an Kohlenstoff gebunden oder gebunden an weiteren Schwefel enthält, von 0,1 bis 10 Gew.-% einer schwachen Säure mit einem pKa von größer als 2 und von 0,05 bis 10 Gew.-% eines Amins enthält, wobei die Prozente auf das Gewicht des Schmiermittels bezogen sind, die Menge an Säure von 0,2 bis 2 Äquivalente pro Äquivalent des Amins beträgt und das Salz der Säure mit dem Amin in dem Schmiermittel löslich ist, in welchem das molare Verhältnis von Schwefel in den Schwefel enthaltenden Höchstdruckadditiven oder Verschleißminderern zu dem Aminostickstoff des Amins von 40:1 bis 5:1 beträgt.

2. Zusammensetzung gemäß Anspruch 1, die 0,67 bis 1,25 Äquivalente der Säure pro Äquivalent des Amins enthält.

3. Zusammensetzung gemäß Anspruch 1 oder 2, welche von 1,7 bis 10 Gew.-%, bezogen auf das Schmiermittel, des Schwefel enthaltenden Höchstdruckadditives oder Verschleißminderers enthält.

4. Zusammensetzung gemäß einem der Ansprüche 1 bis 3, dadurch gekennzeichnet, daß die Schwefelatome in dem bzw. einem Schwefel enthaltenden Höchstdruckadditiv oder Verschleißminderer hochaktiv sind.

5. Zusammensetzung gemäß einem der vorhergehenden Ansprüche 1 bis 4, dadurch gekennzeichnet, daß das bzw. ein Schwefel enthaltendes Höchstdruckadditiv oder Verschleißminderer 30 bis 50 Gew.-% Schwefel enthält.

6. Zusammensetzung gemäß Anspruch 5, in der das Schwefel enthaltende Höchstdruckadditiv oder Verschleißminderer, das Schwefel direkt an Kohlenstoff gebunden oder an weiteren Schwefel gebunden enthält, Schwefel, ein sulfuriertes Olefin, ein sulfurierter Ester, eine sulfurierte Fettsäure oder ein Dialkylpolysulfid ist.

7. Zusammensetzung gemäß Anspruch 6, in der das Mittel sulfuriertes Isobuten ist.

8. Zusammensetzung gemäß einem der vorhergehenden Ansprüche 1 bis 7, dadurch gekennzeichnet, daß mindestens eines der Schwefel enthaltenden Höchstdruckadditive oder Verschleißminderer ein Dialkyldithiophosphat oder ein anderes Schwefel enthaltendes Phosphit oder ein Phosphitester oder Salz ist.

9. Zusammensetzung gemäß einem der vorhergehenden Ansprüche 1 bis 8, die zusätzlich 0,01 bis 3,5 Gew.-%, bezogen auf das Schmiermittel, eines Phosphor enthaltenden Höchstdruckadditivs oder Verschleißminderers enthält.

10. Verfahren gemäß Anspruch 9, dadurch gekennzeichnet, daß das Phosphor enthaltende Mittel ein Mono- oder Dihydrocarbylphosphat oder eine Mischung derselben ist, wobei der Kohlenwasserstoff Alkyl, Alkenyl, Phenyl, Alkylphenyl oder Dialkylphenyl bedeutet.

11. Zusammensetzung gemäß einem der vorhergehenden Ansprüche 1 bis 10, die zusätzlich 0,1 bis 8 Gew.-% eines Alkalimetallborats, bezogen auf das Schmiermittel, enthält.

12. Zusammensetzung gemäß einem der vorhergehenden Ansprüche 1 bis 11, dadurch gekennzeichnet, daß das Amin ein lineares oder verzweigtes aliphatisches, cycloaliphatisches oder ein lineares oder verzweigtes ethylenisch ungesättigtes aliphatisches Amin mit 6 bis 22 Kohlenstoffatomen oder ein Polyethylenpolyamin ist.

13. Zusammensetzung gemäß Anspruch 12, dadurch gekennzeichnet, daß das Amin ein primäres t-Alkylamin, n-Octylamin, Oleylamin oder Triethylentetramin ist.

14. Zusammensetzung gemäß einem der vorhergehenden Ansprüche 1 bis 13, wobei die Säure eine Carbonsäure ist.

15. Zusammensetzung gemäß Anspruch 14, dadurch gekennzeichnet, daß die Säure eine Alkan- oder Alkenmono- oder -di- oder -polycarbonsäure mit 2 bis 54 Kohlenstoffatomen ist.

16. Zusammensetzung gemäß Anspruch 15, dadurch gekennzeichnet, daß die Säure Essigsäure, n-Octansäure (Caprylsäure), Decansäure (Caprinsäure), Myristinsäure, Ölsäure, Linolsäure, Tetrapropenylbernsteinsäure, Azelainsäure, oder dimerisierte oder trimerisierte Linolsäure ist.

17. Zusammensetzung gemäß einem der vorhergehenden Ansprüche, die weiterhin eines oder mehrerer Antioxidantien, Antischaummittel oder Demulgatoren, Dispergiermittel, Detergentien, Mittel zur Verbesserung des Viskositätsindex, Stockpunkterniedriger und reibungsmindernde Additive enthält.

18. Schmiermittelzusatzkonzentrat, das 5 bis 95 % eines oder mehrerer Schwefel enthaltender Höchstdruckadditive oder Verschleißminderer eingeschlossen mindestens ein solches Mittel, das Schwefel direkt an Kohlenstoff gebunden oder an mehr Schwefel gebunden enthält, von 0,5 bis 20 % einer schwachen Säure mit einem pKa größer als 2 und von 1 bis 20 % eines Amins und ein Verdünnungsöl enthält, wobei die Gewichtsprozente auf das Gesamtgewicht des Konzentrats bezogen sind, die Menge der Säure von 0,2 bis 2 Äquivalente pro Äquivalent des Amins, in dem das molare Verhältnis des Schwefels in den Schwefel enthaltenden Höchstdruckadditiv oder Verschleißminderer zu dem Aminostickstoff in dem Amin von 40:1 bis 5:1 beträgt.

19. Schmiermittelzusatzkonzentrat gemäß Anspruch 18, das zu sätzlich 1 bis 50 % eines oder mehrerer Phosphor enthaltender Höchstdruckadditive oder Verschleißminderer enthält.

## Revendications

1. Composition lubrifiante comprenant un lubrifiant, 1,7 à 20 % en poids d'un ou plusieurs agents extrême-pression ou anti-usure contenant du soufre, renfermant au moins un tel agent contenant du soufre lié directement à du carbone ou à du soufre supplémentaire, 0,1 à 10 % en poids d'un acide faible ayant un pKa supérieur à 2 et 0,05 à 10 % en poids d'une amine, lesdits pourcentages étant basés sur le poids du lubrifiant, la quantité dudit acide allant de 0,2 à 2 équivalents par équivalent de ladite amine, et le sel dudit acide avec ladite amine étant soluble dans ledit lubrifiant, le rapport molaire du soufre dans lesdits agents extrême-pression ou anti-usure contenant du soufre à l'azote de groupe amino dans ladite amine allant de 40:1 à 5:1.

2. Composition suivant la revendication 1, contenant 0,67 à 1,25 équivalent de l'acide par équivalent de l'amine.

3. Composition suivant la revendication 1 ou 2, contenant 1,7 à 10 % en poids du lubrifiant, de l'agent extrême-pression ou anti-usure contenant du soufre.

4. Composition suivant l'une quelconque des revendications 1 à 3, dans laquelle les atomes de soufre dans le, ou un, agent extrême-pression ou anti-usure contenant du soufre sont extrêmement actifs.

5. Composition suivant l'une quelconque des revendications 1 à 4, dans laquelle le, ou un, agent extrême-pression ou anti-usure contenant du soufre renferme 30 à 50 % en poids de soufre.

6. Composition suivant la revendication 5, dans laquelle l'agent extrême-pression ou anti-usure contenant du soufre, renfermant du soufre lié directement à du carbone ou à une quantité supplémentaire de soufre, est le soufre, une oléfine sulfurée, un ester sulfuré, un acide gras sulfuré ou un polysulfure de dialkyle.

7. Composition suivant la revendication 6, dans laquelle l'agent consiste en isobutène sulfuré.

8. Composition suivant l'une quelconque des revendications 1 à 7, dans laquelle au moins un des agents extrême-pression ou anti-usure contenant du soufre est un dialkyldithiophosphate ou un autre phosphite ou ester ou sel de phosphite contenant du soufre.

9. Composition suivant l'une quelconque des revendications 1 à 8, qui contient également 0,01 à 3,5 %, en poids du lubrifiant, d'un agent extrême-pression ou anti-usure contenant du phosphore.

10. Composition suivant la revendication 9, dans laquelle l'agent contenant du phosphore est un phosphate de mono- ou dihydrocarbyle ou un mélange de tels composés, dans lesquels ledit groupe hydrocarbyle est un groupe alkyle, alcényle, phényle, alkyphényle ou dialkylphényle.

11. Composition suivant l'une quelconque des revendications 1 à 10, qui contient également 0,1 à 8 %, en poids du lubrifiant, d'un borate de métal alcalin.

12. Composition suivant l'une quelconque des revendications 1 à 11, dans laquelle l'amine est une amine aliphatique linéaire ou ramifiée, une amine cycloaliphatique ou une amine aliphatique à insaturation éthylénique linéaire ou ramifiée ayant 6 à 22 atomes de carbone, ou bien une polyéthylènepolyamine.

13. Composition suivant la revendication 12, dans laquelle l'amine est une tertioalkylamine primaire, la n-octylamine, l'oléylamine ou la triéthylènetétramine.

14. Composition suivant l'une quelconque des revendications 1 à 13, dans laquelle l'acide est un acide carboxylique.

15. Composition suivant la revendication 14, dans laquelle l'acide est un acide mono-, di- ou polycarboxylique alcanoïque ou alcénoïque ayant 2 à 54 atomes de carbone.

16. Composition suivant la revendication 15, dans laquelle l'acide est l'acide acétique, l'acide n-octanoïque, l'acide décanoïque, l'acide myristique, l'acide oléique, l'acide linoléique, l'acide tétrapropénylsuccinique, l'acide azélaïque ou un acide linoléique dimérisé ou trimérisé.

17. Composition suivant l'une quelconque des revendications précédentes, qui contient également un ou plusieurs composés choisis entre des anti-oxydants, des agents anti-mousse ou des agents désémulsionnants, des dispersants, des détergents, des améliorants d'indice de viscosité, des agents abaissant le point d'écoulement et des modificateurs de frottement.

18. Concentré d'additif lubrifiant comprenant 5 à 95 % d'un ou plusieurs agents extrême-pression ou anti-usure contenant du soufre, renfermant au moins un tel agent contenant du soufre lié directement au carbone ou à du soufre supplémentaire, 0,5 à 20 % d'un acide faible ayant un pKa supérieur à 2 et 1 à 20 % d'une amine, ainsi qu'une huile diluante, lesdits pourcentages étant exprimés en poids sur la base du poids total du concentré, la quantité dudit acide allant de 0,2 à 2 équivalents par équivalent de ladite amine, le rapport molaire du soufre dans lesdits agents extrême-pression ou anti-usure contenant du soufre à l'azote de groupe amino dans ladite amine allant de 40:1 à 5:1.

19. Concentré d'additif lubrifiant suivant la revendication 18, qui contient également 1 à 50 % d'un ou plusieurs agents extrême-pression ou anti-usure contenant du phosphore.
